

## UNITED STATES PATENT OFFICE.

HARRY C. CLAFLIN AND ADELBERT SCHADE, OF NITRO, WEST VIRGINIA.

## COMPOSITION OF MATERIAL.

No Drawing.

Application filed May 7, 1921. Serial No. 467,543.

*To all whom it may concern:*

Be it known that we, HARRY C. CLAFLIN and ADELBERT SCHADE, citizens of the United States, residing at Nitro, in the county of

5 Putnam and State of West Virginia, have invented certain new and useful Improvements in the Composition of Material, of which the following is a specification.

This invention relates to a composition of 10 material for general use, and particularly for use as a bearing metal.

An object of the invention is to provide a metal which may be used to form shaft bearings, and the like, and which will 15 provide a bearing capable of efficiently performing its office for prolonged periods without necessity for the usual careful attention given to bearings of this kind.

A further and more detailed object is to 20 provide a bearing metal which will stand up, without danger of overheating or of other injury even if not sufficiently lubricated by the application of oil or other lubricant thereto.

25 A further object is to provide a metal alloy which, while highly efficient as a bearing metal is at the same time capable of use in various other connections as for instance in the manufacture of so-called hard 30 lead pipe, printers type, and for the manufacture of numerous other articles which have heretofore been made up of lead-antimony alloys.

Other objects and aims of the invention, 35 more or less specific than those referred to above, will be in part obvious and in part pointed out in the course of the following description and application of principles constituting the invention, and the scope of 40 protection contemplated will be indicated in the appended claims.

We have discovered that these results may be attained by the use of a main body of lead 45 mixed with a small percentage of metallic magnesium and of metallic sodium. The quantity of magnesium employed may range from two (2) to six (6) per cent of the whole, and the sodium from one (1) to three (3) per cent.

50 The three ingredients named, mixed in the approximate proportions indicated, produces a composition, or alloy, which is of a hard and tough texture, thereby giving ample strength, but which is at the same time suitably smooth to make an excellent bearing.

55 The alloying of the magnesium with the

lead produces a chemical composition which is considerably harder and of increased heat resisting value as compared with the lead alone. The heat resisting value thus imparted to the composition by the addition of the magnesium raises the melting point so that the heat generated, for instance, by a revolving shaft within an insufficiently lubricated bearing, may be maintained for 60 a prolonged period without likelihood of melting or dragging of the bearing. The increased degree of hardness also better adapts the metal to resist the pounds which often occur in journal or bearing boxes. 65

The small quantity of sodium employed is of great importance; first, in that it materially aids in alloying the other two metals; second, that it renders the resultant metal of a clearer and more homogeneous texture; 70 and third, and most important, that it serves to reduce the co-efficient of friction thus reducing the frictional heat generated by the revolving shaft.

Any ordinary scrap lead, or other lead, 75 which is not an alloy, may be employed for this metal. It is first melted in an iron or other suitable container to a temperature only slightly above the melting point, the dross being skimmed off. The magnesium 80 is separately treated in the same manner, and when both metals have been thus heated, the magnesium is poured into the lead. The resultant chemical heat facilitates the mixing which is effected preferably by stirring. 85 While still stirring, the mixture is allowed to cool until when almost at the point of solidification the required amount of metallic sodium is added in the solid state. 90

Before final cooling, the completed alloy 95 thus formed, is preferably poured into suitable moulds.

Thereafter, it may be remelted and poured into bearings, according to the present methods in practice, of pouring bearing metals, 100 or it may be used for other purposes, as for instance, in the making of printers' type, the manufacture of so-called hard lead pipe, or for many of the other uses for which the well known lead-antimony alloy is now commonly employed, the present alloy in these uses being particularly valuable on account of its great strength and toughness. 105

In a test of this alloy, as a bearing metal, it was impossible to heat the alloy to a 110 sufficient degree to cause it to flow, or drag, the shaft was run without lubricant for

fully thirty (30) minutes at a speed of approximately eighteen hundred (1800) revolutions per minute. At the end of the test the shaft remained bright and clean and the bearing was not injured.

Having thus described our invention, what we claim as new and desire to secure by Letters Patent is:—

1. A bearing metal consisting of lead, magnesium and sodium, the proportion of magnesium being from two to six per cent of the whole and the proportion of sodium being from one to three per cent of the whole.
- 15 2. A bearing metal consisting of a mixture of lead, metallic magnesium and metallic sodium, the magnesium and sodium contents each being less than six per cent of the whole.
- 20 3. The herein-described method of producing a bearing metal, which consists in separately melting to a temperature only slightly above their respective melting points, a quantity of lead and a quantity of

metallic magnesium, stirring said melted metals together while allowing them to cool, and then just before solidification placing in the mixture a quantity of metallic sodium.

4. The herein described method of producing a bearing metal, which consists in melting a quantity of lead and a quantity of metallic magnesium, stirring said melted metals together while allowing them to cool, and then before solidification placing into the mixture an ingredient such as metallic sodium.

5. A bearing metal consisting of a mixture of lead, magnesium, and sodium, the lead being in largely predominant amount and the magnesium and sodium being in comparatively smaller but effective amounts.

In testimony whereof we affix our signatures in the presence of two witnesses.

HARRY C. CLAFLIN.  
ADELBERT SCHADE.

Witnesses:

A. M. DOUGLASS,  
D. E. VANARSDALE.